

## UNITED STATES PATENT OFFICE

CHARLES F. NOFTZGER, OF CHICAGO, ILLINOIS

## MATERIAL ADAPTED FOR BEARINGS, AND BEARINGS THEREOF

No Drawing.

Application filed February 14, 1927. Serial No. 168,231.

This invention relates to an improved bearing or a material which is peculiarly adapted for use in bearings and is useful in certain other relations, and to the method of making 5 the same.

In the manufacture of bearings of this new composition I employ a mineral which is, so far as I am aware found only near Buckeye, Arizona. It, however, may be generally described as being of a crumpled or closely folded sericite schist consisting of aggregates of small scales of the sericite, many of which overlap and which can be easily ground or crushed and containing approximately 45% 10 silicon dioxide, 40% aluminum oxide, 8% potassium oxide, 2% calcium oxide, 1% sodium oxide, 1/2% magnesium oxide and 3 1/2% moisture. These proportions are stated as approximate as they vary somewhat in different specimens.

By the words "sericite schist" as used in this specification and in the claims I contemplate this mineral found near Buckeye, Arizona, or its equivalent.

25 This material I grind, crush or otherwise reduce to a powdered or pulverulent condition and mix with a suitable binder, the binder varying considerably according to the uses for which the bearing is intended; that is, 30 whether it is for heavy work or for high speed work.

One method, and the method I claim herein, of manufacturing my improved bearings and bearing material is as follows:

35 The sericite schist is ground or crushed and mixed with a comminuted partial reaction product of phenol and formaldehyde in the proportions of about 60% of the powdered mineral to 40% of such reaction product, the 40 mixture being very thorough.

The mixture is then molded under pressure and subjected to heat which transforms the phenol-formaldehyde product into a fixed or insoluble infusible condensation product.

45 The result is a bearing which is capable of withstanding heavy loads and is of very high antifriction qualities. The proportions may be varied but they are such that the bearing is characterized by the bearing and lubricating qualities of the mineral.

My improved bearings also are well adapted to withstand alkali and other solutions which are detrimental to certain commonly used mineral bearings.

Other binders have been used with this 55 particular mineral with satisfactory results, among such materials being a mixture of litharge and glycerin and the ground mineral, about 35 parts of the litharge and glycerin with 65 parts of ground mineral in bulk, 60 the mixture being subjected to simultaneous heat and pressure. Gum arabic and castor oil in equal parts with a mixture of about four times in bulk of ground mineral, simultaneously heated and subjected to high pressure is highly satisfactory in high speed 65 bearings.

My improved bearings have very excellent 70 wearing and antifriction qualities, do not require lubricant and are adapted for various uses, both high speed and heavy pressure duty.

Having thus described my invention what I claim as new and desire to secure by Letters Patent is:

1. A bearing comprising a pulverulent sericite schist comprising approximately 95% of oxides, and an infusible phenolic condensation product in the proportions of approximately 60% to 80% of the pulverulent sericite schist and 20% to 40% of the phenolic condensation product.

2. A bearing comprising ground sericite schist and an insoluble condensation product of phenolic body, and formaldehyde.

3. A bearing comprising sericite schist comprising approximately 95% of earthy oxides, and a binder, in such proportions that the binder is characterized by the wearing and lubricating qualities of the mineral.

4. A bearing comprising a powdered sericite schist containing approximately 95% of oxides, and a binder, in the proportions of approximately 60% to 80% of the powdered sericite schist and 20% to 40% of the binder.

5. An article of manufacture consisting of pulverulent sericite schist, and a binder, in the proportions of 60% to 80% of the sericite schist and 20% to 40% of the binder.

6. A new article of manufacture consisting

of ground sericite schist, and an insoluble condensation product of phenolic body and formaldehyde.

7. A bearing comprising pulverulent sericite schist incorporated with an insoluble binder in such proportions that the bearing is characterized by the wearing and lubricating qualities of the mineral.

8. A new article of manufacture comprising a pulverized sericite schist, and an insoluble infusible binder, the mineral being intimately mixed or incorporated with the binding material.

9. A composition of matter comprising pulverulent sericite schist and an infusible condensation product in the proportions of approximately 60% of the pulverulent sericite schist and 40% of the phenolic condensation product.

10. A composition of matter comprising a pulverulent sericite schist and an insoluble condensation product of phenolic body and formaldehyde characterized by antifriction or lubricating qualities, resistance to moisture, heat and acids.

In witness whereof I have hereunto set my hand.

CHARLES F. NOFTZGER.

33

40

45

50

55

60